

# United States Patent Office

2,890,143

Patented June 9, 1959

1

2,890,143

## ANNEALING PROCESS FOR MINIMIZING CORE LOSS IN HOT-ROLLED ELECTRIC SHEET SEGMENTS

Jakob Bingel, Berlin, Germany

No Drawing. Application January 11, 1956  
Serial No. 558,604

1 Claim. (Cl. 148—112)

This invention is concerned with a heat treatment of ready stamped sheet segments, in particular of segments for use in dynamo electric machines, with the aim of reducing core loss and increasing the magnetic properties; the segments are annealed in the stack. The invention is most effective as a process for re-annealing stamped segments. The process allows, in the case of sheets with medium silicon contents (1.5%—3.5% Si), magnetic and mechanical properties to be retained, which are not simultaneously present in high silicon sheets. Very low losses are achieved with sheets annealed in this way, and enhanced magnetization, without the necessity of starting with a hard and brittle material with reduced magnetization. The process does not demand the use of high grade electric furnace smelted steel; sheets of cheap Siemens-Martin steel are used. No use is made of grain orientation by cold rolling and thus low core losses and high magnetization in all directions of the sheet are achieved, for which reason the invention is particularly suitable for the treatment of the core material in generators and motors. As the new process does not depend on any metallurgical purification of the core material by quick flowing hydrogen with the object of decarburisation etc., it can be carried out in a static or creeping protective gas, that is in the simplest way under the purest conditions.

This invention is based on new discoveries in the field of metal physics.

Dynamo sheets with silicon contents above 2% are at present stage of technics annealed at about 800° C., for one thing to eliminate the distortion hardenings arising during processing, for another to convert the released carbon into graphite. The simplest method for this box annealing is in air. Box annealing at higher temperatures is deprecated at the present stage of technics, for at 1000° C. a deterioration in the loss figures and mechanical properties becomes noticeable, which is known as over-annealing.

With the present invention electric sheet segments, particularly those intended for dynamo electric machines, can under certain conditions be annealed at much higher temperatures (1100°—1250° C.) with the object of reducing core loss and enhancing magnetization.

It is, of course, known that transformer sheets are annealed at above 1100° C. in a high vacuum, though improvements of quality are only achieved with a vacuum superior to  $10^{-2}$  Torr. in consequence of a crystal purification through pumping out the released and reaction gases from the sheets. This method of increasing the initial permeability is unsuitable for dynamo sheets, for in the vacuum during the high-temperature annealing a brittleness arises in the sheets insupportable for machines, which can not be removed, and again vacuum annealing is not a large-scale technical process.

In connection with the idea of the invention on the other hand it was ascertained on hot-rolled, normally annealed dynamo sheets with 2.4% silicon content after five hours' re-annealing at 1200° C. in argon of 1 atmosphere pressure that the hysteresis loss had sunk from 1.8

2

w./kg. (1.8 watts/kilogramme) to 1.2 w./kg. The simultaneous metallographic test of the annealed material showed, besides a slight coarsening of the grain, the precipitation of large perlite islands, which in the micro-structure of the original sheet could not be discerned even in 100-fold magnification.

The connection between the reduction of hysteresis loss and the appearance of the perlite islands can only be interpreted as being the result of the originally highly dispersed cementite having collected during high-temperature annealing and during the cooling stage precipitating itself as coarse perlite. This provides a new standpoint insofar as according to the "foreign body theory" agglomerations are less harmful magnetically than highly dispersed distributions and so reduce coercive force and with it hysteresis loss. If following the above mentioned theory the coercive force  $H_c$  is represented in the form

$$H_c = C \frac{\delta}{d}$$

in which C is a constant and

$$\frac{\delta}{d}$$

is the relation of the "Blochwall"  $\delta$  in the Weiss magnetic elementary area to the size of particle  $d$ , it will be seen that with increasing coagulation of the foreign bodies the coercive force rapidly sinks.

In contrast to the usual view held by metallurgists, who regard elimination of carbon and other foreign elements by chemical reactions from the sheet as the sole prerequisite for reducing hysteresis loss, there is shown here the effect of a "collective precipitation" at the grain boundaries, brought about by diffusion during a lengthy anneal at 1200° C.

At the same time it was possible to prove that the silicon content within narrow limits plays a considerable part in precipitation insofar as an anneal at the same temperature on low-silicon dynamo sheets produces a much smaller result with regard to lowering hysteresis loss than with high-silicon sheets. As it is known that silicon promotes crystallization and so accelerates the displacement of the foreign elements to the grain boundaries, the enhanced influence of the silicon on collective precipitation can be explained. As diffusion processes increase with rising temperature, annealing temperatures of 1200°—1250° C. are recommended for low-silicon sheets, for very high-silicon sheets 1100° C. So on dynamo sheets with 3.2% silicon content it was possible to achieve a hysteresis loss of 0.7 w./kg. at 1200° C. after 10 hours, during which time monocrystals of 10 mm. diameter had formed in the sheet.

As a result of the annealing the magnetization also increases at all field strengths by 400 gauss.

The process can also be applied on segments which have been cut out from unannealed panels, so long as the panels have been given an absolutely even surface by finishing.

As high-temperature annealing in a slowly flowing gas has the same effect as in a stagnant protective gas, it can be used as a technical process, for the speed of flow can be reduced at will so as to substitute a creeping gas flow for the stagnant gas.

In the light of the invention it is suggested that segments of hot-rolled dynamo electric sheets should be annealed in slowly flowing, technically pure argon, hydrogen, or nitrogen at temperatures between 1100° C. and 1250° C. for several hours.

The slow flow is a necessary condition, for otherwise undesirable foreign gases such as oxygen and water vapour would be drawn into the container and oxidation

could take place. This condition, however, also suffices for the purpose of collective precipitation, for it is not aimed at chemical purification, which for the purpose of drawing off reaction gases demands high flowing speeds.

For this reason the new method is not identical with the similar well-known process which by annealing of ferrosilicon alloys in chemically pure hydrogen with high speed of flow between 1100° C. and 1400° C. achieved high initial permeabilities, which call for absolute purity of the material. It is known that decarburization in electric sheets at high temperatures can only be achieved in quickly flowing hydrogen, for the reaction



at a high temperature only becomes effective through constant disturbance of the equilibrium, whereas with slower flow the equilibrium is shifted far to the left and no decarburization takes place.

As a further result of the invention oxidation of the sheets over a short period by oxygenous nitrogen can after cooling to 800° C. be of particular importance, in that by a chemical attack it again neutralizes the brittleness of the sheets.

The practical operation of the process consists appropriately in arranging the sheet segments separated by  $Al_2O_3$ -powder, in several stacks in an iron container welded or riveted hermetically; an inlet and an outlet pipe are welded to the container, through which the gas flows. The gases developed during heating up pass out through the outlet, while the inlet is closed. From 900° C. onward intermittent cleansing with argon is carried out for a short period, which can cease at 1200° C. when the container has been sealed. To counteract warping of the sheet segments it is advisable to use weight plates suitably arranged in the stacks. A further artifice consists in applying a directed flow, driving the desired gas on to every point of the surface inside the sheet pile. Finally the hood furnace has proved useful for heating; it can, alternately with cooler hoods, be propped over the various containers on ceramic pillars, whereby a continuous annealing program can be maintained.

It is a matter of course that the annealing container can be used repeatedly when surrounded by a cheap protective gas and kept free from scale.

There is today in electro-mechanical engineering a demand for dynamo sheets with extremely low core loss. The direct way to achieve this is by re-annealing the stamped machine segments at 1100° to 1250° C., which not only eliminates cut-hardening but at the same time has an improving effect on the crystal structure of the iron. In contrast to transformer cores, stamping reintroduces into the deeply incised machine segment with long teeth and wide guide holes, greater tensions, which as cut-hardening again enhances hysteresis loss. At the edges of the cut the coercive force is greatly increased, on the other hand the mean tooth induction is very high, so that in segments with narrow teeth a rise in total core

loss of the segment of 15%, in those with wide teeth of 10% is calculated. For this reason it has already been suggested subjecting the stamped segments to a stress-relieving anneal at 700° C.; this procedure is, however, not economical enough and for that reason alone has never been introduced.

According to the invention, the total reduction in core loss is 45%.

This way of re-annealing stamped segments at very high temperature could only be proposed once it had been proved that the expansion due to heat is reversible and also that no appreciable changes in length remain as a result of the precipitations caused and of the equalization of tension brought about. In practice accuracy of size of  $\pm 0.01$  mm. in tooth breadth and  $\pm 0.3$  mm. in segment length is called for, for after assembly a smooth slot surface must essentially be present to take the conductor.

With the aid of microscope micrometers with an accuracy to 1 micron, it was established both on 200 mm. check gauges and on segments, that annealing at 1200° C. causes a shrinkage of only  $1.5 \cdot 10^{-2}\%$  as long as the panel has been normalized in the rolling mill at 800° C., and a shrinkage of  $3 \cdot 10^{-2}\%$  without normalizing having been done. This proves that high-temperature annealing of segments does not influence the accuracy in size of machine construction and the original dimensions are retained in the slot within limits of  $\pm 0.01$  mm.

I claim:

30 A heat treatment for stacks of hot-rolled silicon steel electric sheets for generators to produce segments with very low hysteresis losses and good mechanical properties, which treatment comprises annealing ready stamped segments with a silicon content of 1.5%-3.5% in an industrial protective gas between 1100° and 1250° C. for several hours, and then cooling the stack to about 800° C., and then oxidizing the segments for a short time in a stream of strongly oxidizing gas.

#### References Cited in the file of this patent

#### UNITED STATES PATENTS

|           |                |               |
|-----------|----------------|---------------|
| 1,569,355 | Cole           | Jan. 12, 1926 |
| 2,158,065 | Cole et al.    | May 16, 1939  |
| 2,209,684 | Crafts         | July 30, 1954 |
| 2,599,340 | Littman et al. | June 3, 1952  |

#### OTHER REFERENCES

The Electric Journal, vol. 21, pages 55 to 61. Published in 1924 at Pittsburgh, Pa.

50 Stahl and Eisen: Vol. 48, pp. 484 and 485. Publ. in 1928.

55 Alloys of Iron and Silicon, 1st edition, pp. 355 and 356. Edited by Greiner, Marsh and Stoughton. Published in 1933 by the McGraw-Hill Book Co., New York, N.Y.

Ferromagnetism, pp. 92 and 93. Edited by Bozorth. Published in 1951 by D. Van Nostrand Co.